

K. SUNDBERG,  
SELECTIVE FLOTATION OF MINERALS,  
APPLICATION FILED MAR. 19, 1918.

1,326,545.

Patented Dec. 30, 1919.



FIG. 2.



INVENTOR:

Karl Sundberg,  
By  
Mr. Wallace White

ATTY.

# UNITED STATES PATENT OFFICE.

KARL SUNDBERG, OF STOCKHOLM, SWEDEN.

## SELECTIVE FLOTATION OF MINERALS.

1,326,545.

Specification of Letters Patent.

Patented Dec. 30, 1919.

Application filed March 19, 1918. Serial No. 223,380.

*To all whom it may concern:*

Be it known that I, KÄRL SUNDBERG, a subject of the King of Sweden, residing at Stockholm, Sweden, have invented certain new and useful Improvements in Selective Flotation of Minerals, of which the following is a specification.

My invention refers to a process of separating from a mineral, for instance an ore or a small ore, containing one or more floatable minerals, each of these minerals *per se*. With the term "floatable minerals" I mean such minerals which in mixture in a finely divided state with a liquid and foam producing means, after forcing air or another gas through the mixture are raised with the foam produced to the surface of the mixture. The process is practicable for instance for the separation of galena and zinc-blende in a small ore containing these minerals, specular iron ore and copper pyrite in a cuprous red hematite ore, or galena, zinc-blende and copper pyrite in a small ore containing these minerals.

The invention is based upon the different disposition of the different minerals to rise with the foam produced, in such a manner that in the treatment of an ore containing several minerals in a flotation apparatus with several compartments or chambers the foam in the first chamber or chambers will contain essentially greater quantities of the more floatable mineral than of the other one, which latter mineral will accumulate in the foam, produced in the last chamber or chambers. In fact the proportion of the quantities of the different minerals in the foam from the different chambers can be determined once for all, because under for the rest equal circumstances this proportion is proportional to the proportion of the mineral components of the material to be treated in the apparatus. If thus in the treatment in a flotation apparatus with several chambers of an ore mixture, containing 25% of each of two minerals, the foam in the first chamber contains 50% of the one and 5% of the other mineral, the proportion of the minerals in the foam in the treatment of an ore mixture containing 30% of the first mentioned mineral and 10% of the mineral last mentioned becomes  $\frac{30 \cdot 50}{5 \cdot 10} = 30 : 1$  in place of the proportion 50 : 5 first mentioned.

The invention consists therein that the mineral mixture in the usual manner is

floated in a flotation apparatus with several chambers or compartments, whereupon the foam from the first and last chamber or from some of the first and the last chambers of this apparatus (the said foam thus containing either of the minerals in a great quantity) is brought respectively into the first chamber of two other flotation apparatus where it is floated anew and the product thus obtained from the first chamber of the one of these apparatus and from the last chamber of the other apparatus is let off and collected, while the foam from the intermediate chambers of the flotation apparatus is brought back to the first chamber of the apparatus first mentioned or to the first chambers in each apparatus and then submitted again to flotation.

In the accompanying drawing Figures 1 and 2 are schematic views showing two processes embodying my invention. The process illustrated in Fig. 1 is applied to a material containing two minerals in equal proportions. For carrying out the process at first for instance three apparatus divided in five chambers or compartments *a*, *b*, *c*, are used. In the flotation in the apparatus *a* the two minerals distribute themselves in the foam for instance in the proportion 1:4 in the first chamber, 1:2 in the second chamber, 1:1 in the third chamber, 2:1 in the fourth chamber and 4:1 in the fifth chamber, as shown in the drawing. From the first chamber of the apparatus *a* the foam produced is carried to the first chamber of the apparatus *b*, where a concentration of the mineral easiest to float takes place. This mineral, which now is very pure from the other one (for instance in the proportion 16:1) is removed, and the remaining mineral is floated in the other chambers of the apparatus *b*. The foam produced by this latter flotation as also the foam obtained in the chambers 2-4 of the apparatus *a* is brought back to the first chamber of the said apparatus *a* or to the first chamber of the apparatus *b* and again submitted to flotation. In the same manner the foam from the last chamber 5 of the apparatus *a* is brought to the first chamber of the third apparatus *c*, where it is floated again. From the last chamber 5 of that apparatus the foam rich in the second mineral is removed, while the foam from the other chambers in the apparatus *c* is brought to the first chamber of the apparatus *a* or to the first chamber of the apparatus *c*,

The foam from an intermediate chamber 3 in the apparatuses *b* and *c* can also be brought back to the first chamber 1 in these apparatuses in place of to the chamber 1 in the apparatus *a*. In Fig. 1 the approximate proportions of the minerals at different stages of the flotation is shown, and the courses in which the foam is brought from the different apparatus are marked 10 with arrows.

In this way a separation of the minerals can be produced, so that the small ore from the first chamber of the apparatus *b* contains 16 parts of the one mineral against 1 part 15 of the other one, while the small ore from the last chamber of the apparatus *c* contains 1 part of the mineral first mentioned on 16 parts of the other one. By using still more flotation apparatuses a further concentration 20 of course is obtainable.

Fig. 2 illustrates, also schematically, the process applied to a material, containing three minerals of different adaptability for flotation. In this case more apparatuses *a*, 25 *b*, *c*, *d*, *e*, *f* than now described are used.

The ore is first floated in the apparatus *a*, whereby the foam from the first chamber of this apparatus is brought into the first chamber of the next apparatus *b*, while the foam 30 from the last chamber of the apparatus *a* is brought into the first chamber of the apparatus *c*. The foam from the other chambers 2-4 of the apparatus *a* is brought back to the first chamber of this apparatus and 35 floated again. The foam from the first chamber 1 in the apparatus *b* (which foam contains the mineral easiest to float) is collected and the foam from the last chamber 5 of the same apparatus *b* is brought to the 40 first chamber 1 of an apparatus *e*, while the foam from the intermediate chambers 2-4 of the apparatus *b* is brought back to the first chamber 1 of the apparatus *b* or the first chamber of the apparatus *a*, where it is 45 again submitted to flotation. In the same manner the foam from the first chamber of the apparatus *c* is brought into the first chamber of the apparatus *e*, while the foam from the last chamber 5 of the apparatus *c*, 50 which foam is rich in the mineral most difficult to float, is removed and collected. The foam from the intermediate chambers 2-4 of the apparatus *c* is brought back to the first chamber of the apparatus *a* or *c*, the 55 foam from the latter as also from the last chamber of the apparatus *b* containing more of the mineral having an adaptability for flotation between that of the two other minerals. In the apparatus *e* the foam is again 60 floated and is then from the first chamber of the said apparatus brought to the first chamber of the apparatus *d*, from which chamber the foam rich in material easy to float is removed and collected together with 65 the material from the first chamber 1 of

the apparatus *b*, forming a small ore rich in the said mineral. From the last chamber 5 of the apparatus *e* the foam rich in the mineral most difficult to float is brought to the first chamber of the apparatus *f*, where it is 70 floated again, and from the last chamber 5 of the said apparatus the foam, rich in the mineral most difficult to float is removed and collected together with that from the last chamber of the apparatus *c*. As well in the 75 apparatus *d* as in *e* and *f* the foam from the chambers 2-4 is brought back to the chamber 1 in each such apparatus. The mineral with a floatability between that of the two other minerals, is contained in the foam obtained in the last chamber of the apparatus *d* and the first chamber of the apparatus *f*, for which reason that foam is removed separately, so that the said mineral can be collected from the foam. Of course it is possible also in the process now described to complete the enriching of the minerals from the ore, by increasing the number of apparatus used. 80 85

From the examples given it is evident, 90 that according to the present invention it is always possible in the flotation apparatuses with several compartments or chambers to separate the floatable components of the material by floating anew the foam from the 95 first and last chamber or chambers *per se* in other flotation apparatuses, in which the foam from the first chamber of the one apparatus and from the last chamber of the other apparatus is collected as a finished 100 product or is again floated in other apparatuses, while the foam from the intermediate chambers (between the first and the last chamber or chambers) is floated again in the same or in a preceding apparatus. 105

Having now particularly described the nature of my invention and the manner of its operation, what I claim is:

1. A process for separating minerals by flotation which consists in pulping the ore; 110 treating the same in flotation apparatuses with several compartments in such a manner that the foam from the first compartment and that from the last compartment of one apparatus is floated again *per se* in 115 a further flotation apparatus, while the foam from the intermediate compartments of each apparatus after the initial treatment apparatus is brought back to and floated in the first compartment in one of the flotation apparatuses. 120

2. A process for separating minerals by flotation which consists in pulping the ore; 125 treating the same in flotation apparatuses with several compartments in such a manner that the foam from the first compartments and that from the last compartments of one apparatus is floated again *per se* in a further flotation apparatus, while the foam from the intermediate compartments of each apparatus 130

ratus is brought back to and floated in the first compartment in one of the flotation apparatus, and the material which has not been taken up by the foam from the last 5 compartment of the first apparatus is brought to and floated in a second apparatus, whereupon the foam produced at this flotation is collected together with that previously obtained and submitted to repeated

flotations, the non-floatable material remaining being collected *per se*.

In testimony whereof I have affixed my signature in presence of two witnesses.

KARL SUNDBERG.

Witnesses:

S. MAGNUSSON,  
H. TELANDER.